

# UNITED STATES PATENT OFFICE.

ANDREW MUHA, OF CLEVELAND, OHIO.

## CLEANSING AND POLISHING COMPOSITION.

1,342,862.

Specification of Letters Patent.

Patented June 8, 1920.

No Drawing.

Application filed October 24, 1919. Serial No. 332,905.

*To all whom it may concern:*

Be it known that I, ANDREW MUHA, a citizen of Austria, now Jugoslavia, residing at Cleveland, in the county of Cuyahoga and State of Ohio, have invented certain new and useful Improvements in Cleansing and Polishing Composition, of which the following is a specification.

The invention herein consists in a composition for cleansing and polishing various surfaces, such as highly polished automobiles, pianos, graphophones and other furniture and articles susceptible of a polished finish, and the said composition is of such quality that it serves also as a perfect cleansing medium which will not discolor nor produce a stain or other injury or blemish, and, when applied according to directions, will leave the surface clean with a polish that has all its original luster or brilliancy and is devoid of gummy or like condition which would gather dust and be objectionable on this account.

In carrying out my invention and for the production, say of about a gallon of the mixture, I employ the following ingredients in about the proportions stated:

2 quarts of lubricating or linseed oil.

2 " of pure water.

30 2 ounces of spirits of turpentine.

2 " of cider vinegar.

2 " of alcohol.

2 " of oil of citronella.

4 " of butter of antimony.

35 The vinegar imparts a quick cutting or cleansing action to the composition; however, the vinegar may be omitted if desired. These ingredients are such that they

can be mixed cold, if preferred, or they may be more or less warmed to promote 40 admixture, and the finished product will be practically homogeneous and adapted to be poured like a creamy liquid. Any tendency to settle by long standing can easily be overcome by shaking the bottle or vessel, 45 and the application is made by cheesecloth or the like with rubbing, care being taken that the cloth is such that it will not scratch or mar the surface. Furthermore, if the surface is covered with gritty matter or 50 sand, as is liable to be the case with automobiles, it should be first thoroughly washed and cleansed in this particular. Then after drying the surface the compound can be applied with safety and effectiveness for giving a superior gloss which holds like the original polish.

Wood alcohol can be used for economy.

What I claim is:

1. The herein described composition for 60 cleansing and polishing various surfaces comprising a heavy oil, water, spirits of turpentine, alcohol, oil of citronella, and butter of antimony.

2. The herein described composition of 65 matter for cleansing and polishing comprising a heavy oil, two quarts; pure water, two quarts; spirits of turpentine, two ounces; alcohol, two ounces; oil of citronella, two ounces; and butter of antimony, four 70 ounces.

Signed at Cleveland, in the county of Cuyahoga and State of Ohio, this 18th day of October, 1919.

ANDREW MUHA.